

Oct. 28, 1941.

W. E. ROBBINS ET AL

2,260,683

PROCESS OF INHIBITING THE OXIDATION OF HYDROCARBONS

Filed Sept. 7, 1939



Inventors: Wilbur E. Robbins  
Richard R. Zundel  
By their Attorney: E. W. Dubois

## UNITED STATES PATENT OFFICE

2,260,683

PROCESS OF INHIBITING THE OXIDATION  
OF HYDROCARBONS

Wilbur E. Robbins, Norco, La., and Richard R. Zundel, Wood River, Ill., assignors to Shell Development Company, San Francisco, Calif., a corporation of Delaware

Application September 7, 1939, Serial No. 293,708

5 Claims. (Cl. 44—9)

This invention relates to a process of inhibiting oxidation of hydrocarbons by the use of alkyl phenols as anti-oxidants and gum inhibitors and more particularly is concerned with the use of certain fractions of crude alkyl phenols in hydrocarbon oils as anti-oxidants and gum inhibitors which have a greater effectiveness in this function than the ordinary bulk alkyl phenols.

Alkyl phenols from various sources such as petroleum and coal tar, and various distillation cuts of these alkyl phenols have been used as anti-oxidants in gasolines and the like. However despite the fact that these inhibitors are readily available and inexpensive, their use has been greatly limited because of the fact that a comparatively large quantity must be added to secure the inhibiting effect produced by a much smaller quantity of many other inhibitors such as amino phenols, aromatic diamines, etc. It is an object of this invention to provide alkyl phenol fractions of high inhibiting value which may be inexpensively and easily prepared from crude alkyl phenols or their distillation fractions of ordinary inhibiting value or from some readily available source of alkyl phenols such as petroleum or coal tar fractions.

It has already been suggested fractionally to distill alkyl phenol fractions and to select those fractions for inhibiting purposes which are most active. However, while there may be some differences in the effectiveness between various fractions so obtained, these differences are normally very small and insignificant.

Now we have found that the relatively weakly acidic alkyl phenols are more effective as inhibitors than the more strongly acidic alkyl phenols having similar boiling points or approximately the same molecular weights, and that the effectiveness as inhibitors of the mixtures of the alkyl phenol fractions rises rapidly with decreasing acidity.

The superior inhibiting effect of the more weakly acidic alkyl phenols can be observed under various conditions, and does not seem to be specific to the stabilization of certain types of materials. In general, wherever alkyl phenol mixtures are active anti-oxidants, the more weakly acidic portions of the mixture are more active than the total mixtures. This applies to the stabilization of hydrocarbon oils, such as cracked gasolines, rubber, paints, etc.

The weakly acidic fractions may be prepared inexpensively and conveniently by fractional ex-

traction of crude alkyl phenol mixtures with caustic alkali such as aqueous solutions of sodium hydroxide, the more strongly acidic fractions being extracted by the caustic alkali forming extracts, and the more weakly acidic ones forming raffinates. By crude alkyl phenol mixture is meant a mixture consisting predominantly of alkyl phenols boiling above about 180° C. which may contain substantial amounts of impurities such as thiophenols and which has been obtained from coal tar or petroleum distillates by extraction with strong aqueous caustic alkali and acidification of the extract. A preferred method for producing crude alkyl phenol mixtures is described in U. S. Patent 2,134,390 by Greensfelder et al. According to this patent alkyl phenols are recovered from hydrocarbon distillates containing them, by treating with aqueous solutions of alkali metal hydroxides having concentrations between 30 and 50% and acidifying the resulting aqueous layer to liberate the alkyl phenols. If desired alkyl phenols may be extracted from distillates by treatment with aqueous caustic solution containing solubilizers such as salts of lower fatty acids having from 2 to 6 carbon atoms, poly-hydroxy alcohols having a greater number of carbon atoms than polar radicals, etc.

The separation of even a small amount of the most strongly acidic components from the crude alkyl phenol mixtures often may cause a marked increase in inhibiting value of the resulting raffinate. Most crude alkyl phenols, and especially those derived from petroleum, normally contain appreciable quantities of thiophenols which usually have a decided detrimental effect on the inhibiting value of the alkyl phenols. Further removal from the crude alkyl phenol mixture of successive quantities of relatively strongly acidic fractions leaves raffinates of increasing inhibiting value. Generally in order to obtain raffinate fractions of greatest inhibiting value it is desirable to recover as a raffinate not more than about half of the total crude alkyl phenols. Such raffinate fractions may have inhibiting values up to four or even more times those of the crude phenols from which they were extracted.

The fractional extraction to separate the crude alkyl phenol mixture into fractions of differing inhibiting powers may be carried out as a counter-current or crosscurrent process and, if desired, in the presence of a substantially water-insoluble solvent for alkyl phenols. The former method is generally advantageous when produc-

ing one fraction of high inhibiting value from sources having rather large amounts of impurities while the latter is often best adapted, where several cuts may be taken from a crude mixture which contains smaller amounts of impurities. 5 However, crude alkyl phenol mixtures are normally exceedingly complex systems, so that with crude alkyl phenols from different sources, it may be necessary to determine experimentally the type of extraction best suited to the particular source, as well as the most economical amount to be recovered as raffinate.

While the effectiveness of the alkyl phenols as anti-oxidants and gum inhibitors is most dependent upon the relative acidity of the fractions, it may also depend to some degree on the boiling range. Thus we have found that the weakly acidic alkyl phenol fractions separated from an alkyl mixture having a boiling range between about 210° to 270° C. are usually more effective than the fractions extracted from other distillation cuts. It is further often advantageous in separating the weakly acid alkyl phenols according to their acidity first to divide the crude alkyl phenol mixture into various distillate fractions of narrow boiling ranges, preferably covering not more than about 20° C., and then separating the several weakly acidic fractions. The latter may be used separately or combined for inhibiting purposes. By this method it is often possible to secure the greatest yield of alkyl phenols having the highest inhibiting value possible from a given crude mixture.

The following is an example of a fractional extraction of crude alkyl phenols, showing the inhibiting values of the weakly acidic fractions to be much higher than those of the bulk alkyl phenols or their more strongly acidic fractions:

Bulk or crude alkyl phenols, obtained by extraction with 40° Bé. caustic soda from a Mid-Continent cracked gasoline having a boiling range of 40° to 200° C., were separated into 15 cuts of successively decreasing acidities by fractional extraction as follows:

A solution of 1200 ml. of the bulk alkyl phenols in 4000 ml. of peroxide free diisobutylene was extracted in six successive extractions with six 250 ml. portions of 5° Bé. sodium hydroxide solution, and the remaining portion was then treated with an amount of an aqueous solution of 50° Bé. sodium hydroxide containing an excess of hydroxide, whereby a phenolate solution was obtained. In the first and second extractions only two layers were formed, but in the third through the sixth extractions three layers were obtained. The six lower extract layers containing the most strongly acidic alkyl phenols were separated and acidified, and the liberated phenols were designated as cuts 1 through 6. The four middle layers consisting of mixtures of water, free alkyl phenols and diisobutylene were treated with 10° Bé. sodium hydroxide to remove diisobutylene, the resulting aqueous layers were acidified and the alkyl phenols so obtained were designated as cuts 7 through 10.

The 50° Bé. phenolate solution was then acidified, the alkyl phenols so liberated were redissolved in 1200 c. c. of diisobutylene and the resulting solution was extracted with five successive 100 c. c. portions of 10° Bé. sodium hydroxide. The alkyl phenols liberated from the five caustic portions constituting the most weakly acidic fractions were designated as cuts 11 through 15. Only a trace of phenols remained in the diisobutylene.

The effectiveness as gum inhibitors of the various cuts is shown in the following table:

| Cut No.      | Increase of induction period in hours on addition of inhibitor to peroxide-free diisobutylene |                                          |
|--------------|-----------------------------------------------------------------------------------------------|------------------------------------------|
|              | Addition of 2 mg./100 gms. diisobutylene                                                      | Addition of 5 mg./100 gms. diisobutylene |
| 15           |                                                                                               |                                          |
| 1            | 7                                                                                             | 1.2                                      |
| 2            | 7                                                                                             | 1.5                                      |
| 3            | 1.0                                                                                           | 2.2                                      |
| 4            | 1.7                                                                                           | 3.0                                      |
| 5            | 2.5                                                                                           | 4.5                                      |
| 6            | 3.2                                                                                           | 6.3                                      |
| 7            | 3.5                                                                                           | 8.0                                      |
| 8            | 3.7                                                                                           | 8.0                                      |
| 9            | 3.5                                                                                           | 8.5                                      |
| 10           | 3.7                                                                                           | 9.0                                      |
| 11           | 3.2                                                                                           | 7.3                                      |
| 12           | 3.7                                                                                           | 8.7                                      |
| 13           | 4.3                                                                                           | 9.7                                      |
| 14           | 6.0                                                                                           | 12.5                                     |
| 15           | 12.3                                                                                          | 25.0                                     |
| Bulk phenols | 3.5                                                                                           | 7.5                                      |

The above example is further illustrated in the drawing in which the anti-oxidant effects of the various cuts are shown graphically. As a reference point, the anti-oxidant effect of 1,2,4,xylene, a well-known antioxidant, under the same conditions is shown.

We claim as our invention:

1. In the process of inhibiting the oxidation of a hydrocarbon susceptible to oxidation and capable of being inhibited with alkyl phenols the steps of extracting a mineral oil containing alkyl phenols and thiophenols naturally occurring therein, with strong aqueous caustic alkali thereby producing an alkyl phenol mixture containing thiophenols, reextracting said mixture with a weaker aqueous caustic alkali solution to form two layers, an extract layer containing the aqueous caustic alkali solution of thiophenols and strongly acidic alkyl phenols, and a raffinate layer substantially free from thiophenols and comprising the more weakly acidic alkyl phenols, and adding a small amount of said raffinate to the hydrocarbon.

2. In the process of inhibiting the oxidation of hydrocarbons susceptible to oxidation and capable of being inhibited with alkyl phenols, the steps of extracting with relatively weak aqueous caustic alkali a mixture of alkyl phenols naturally occurring in mineral oils and having been separated therefrom by extraction with strong aqueous caustic alkali, to produce an extract containing relatively strongly acidic alkyl phenols and a raffinate containing relatively weakly acidic alkyl phenols, and adding a small amount of said raffinate to said hydrocarbons.

3. In the process of inhibiting the oxidation of hydrocarbons susceptible to oxidation and capable of being inhibited with alkyl phenols, the steps of extracting with relatively weak aqueous caustic alkali, a mixture of alkyl phenols having a boiling range of 210° C. to 270° C., naturally occurring in mineral oils and having been separated therefrom by extraction with aqueous caustic alkali of about 30% to 50% concentration to produce an extract containing relatively strongly acidic alkyl phenols and a raffinate containing relatively weakly acidic alkyl phenols and adding a small amount of said raffinate to said hydrocarbons.

4. A composition of matter comprising a hy-

drocarbon oil and an added amount of an alkyl phenol fraction, said fraction comprising a relatively weakly acidic portion of a crude mixture of alkyl phenols naturally occurring in mineral oils and having been separated therefrom by extraction with strong caustic alkali, said fraction having been obtained by fractionally extracting said mixture with weaker aqueous caustic alkali.

5. A composition of matter comprising a hydrocarbon oil and an added amount of an alkyl phenol fraction separated from a crude alkyl

phenol mixture naturally occurring in mineral oils and having been separated therefrom by extraction with strong caustic alkali, said mixture having a boiling range of from 210° C. to 270° C., said fraction having been obtained by extracting said mixture with a weaker aqueous solution of a caustic alkali and being more weakly acidic than the average of said mixture.

WILBUR E. ROBBINS.  
RICHARD R. ZUNDEL.